

1

3,814,597

## ABRASION RESISTANT CAST FERROUS ALLOYS

Samuel A. Sholl, Clearfield, Pa., assignor to Clearfield Machine Company, Clearfield, Pa.

No Drawing. Filed Sept. 27, 1971, Ser. No. 183,876  
Int. Cl. C22c 37/00, 37/100

U.S. Cl. 75—123 CB

5 Claims

### ABSTRACT OF THE DISCLOSURE

A new cast iron and article of manufacture made therefrom is provided having unusual abrasive resistance and an oriented lamellar structure consisting of at least one member from the group pearlite and bainite and a complex carbide structure consisting of boron nitrides, boron carbides and other boron compounds.

The present invention relates to cast ferrous alloys and particularly a unique ferrous alloy having an exceptional combination of physical properties including outstanding resistance to abrasion, air hardening and wear resistance. The alloy is of special utility in the manufacture of articles which are used in grinding or polishing or in handling abrasive material such as sand, shot or the like.

In general, regular cast iron, with ladle additions of such elements as chromium, molybdenum, nickel and copper either singly or in combinations with other elements are used to produce an improved abrasion or wear resistant cast iron. These elements will impart a matrix structure containing a portion of complex carbides, ferrite, pearlite, together with flake or nodular graphite. The type or form of graphite depends upon the process used in producing the alloy. In addition to these elements cited above, the addition of increased manganese percentages is also beneficial as an assist towards further improvement in the wear resistant properties. When the manganese content is increased above that normally contained in cast iron, range from about 0.30 to 1.00%, the manganese has the property of imparting to the ferrous alloys improved wear resistance when in contact with granular hard mineral substances. As in all ferrous castings, the percentages of the elements mentioned above are related to the thickness of the castings and the rapidity of the air quench as the castings are cooled below the critical temperature. Depending upon the gradient temperature, hard massive carbides will be developed to a greater or lesser degree in the metals' matrix structure. In addition, the reduction in the percentages of carbon and silicon will have a profound influence on the amount of carbide produced and will have a direct bearing upon the toughness or brittleness of the metal to such an extent that the castings will become excessively brittle and break upon the slightest rough handling. In these types of cast iron, the massive carbides are randomly oriented throughout the matrix structure and do not have the tough resistance to abrasive wear to obtain satisfactory life, when exposed to minerals having a hardness of more than 5 on the Mohr's hardness scale.

The present invention is based upon the discovery that the element boron when used in conjunction with other elements in proper amounts, in ferrous alloys where free carbon is present, such as the cast irons which are either hypo or hyper eutectic, will produce a superior abrasion wear resistant alloy iron that is superior in many aspects to the present family of cast irons of this type. In the ferrous alloy of the invention boron and manganese and other elements such as enumerated above, are added to the melt in sequence, so as to provide a family of nodular and flake irons that will produce a directionally oriented matrix structure consisting but not necessarily adhering to plate carbides of complex type and more or less alternating with pearlite or bainite.

2

It is an object of this invention to provide a ferrous alloy of superior abrasion and wear resisting properties.

Other objects and advantages of the present invention will be apparent to those skilled in the art from the following description and the figures of photomicrographs shown.

The present invention provides an unique and novel ferrous product containing at least 40% carbon and silicon within the cast iron range, and at least 0.1% boron, and at least 0.30% manganese. Free carbon may be in small amounts of vermicular, nodular, or flake form. The ratio of the complex carbides to pearlite remains in approximately 1 to 1 proportions for all applications, but adjustments in elemental content will vary according to the metal thickness and mass involved. This structure is obtained in the "as cast" condition. No heat treatment is required, a definite advantage over those requiring heat treatment to obtain the necessary properties.

Both manganese and boron have been used extensively in the founding art. But the combination of these two to produce the type of ferrous alloy described has not been known to be used. The use of elemental manganese in excess of approximately 1% often is conducive to producing gas hole defects in castings, caused, it has been postulated, by either molecular hydrogen or molecular nitrogen in cast iron.

With the addition of boron to the melt this problem of gas hole casting defects has been eliminated, due probably to the boron reacting stoichiometrically with atomic hydrogen or atomic nitrogen to form complex boron hydrides and boron nitrides in the presence of the high energy developed in the molten metal. The boron nitrides are exceedingly hard and approach the diamond in hardness. Therefore, minute quantities of these boron compounds located in interstitial positions within the body centered cubic structure of the ferrous metal materially assist in imparting increased resistance to abrasion and other wear resisting properties. The interstitial compounds thus formed have the properties of true metals, and have the formula of the MX type.

The interstitial compounds, in addition to those described above, and incorporated into the cubic structure are other borides including manganese boride, ferrous borides, silicon boride, and boron carbides. These compounds are also extremely hard with hardness values lying between diamond (10) Mohr's scale and Topaz (8). It is, therefore, probably these metallic compounds that cause the unique properties described above. But in addition to this I have found that the alloy has uniqueness of orientation of the carbides and nitrides alternating with a pearlitic, bainitic oriented matrix structure that also imparts toughness to the metal. The apparent alternation of these plates causes these properties to occur, that is toughness in conjunction with wear and abrasion resistance.

This invention can perhaps best be understood by reference to the following examples.

### EXAMPLE I

Muller wear plates for crushing large pieces of minerals such as bauxite, kaolinite, quartz and calcined clay were made by casting from the following alloy composition:

|                | Percent |
|----------------|---------|
| C              | 3.40    |
| Si             | 2.40    |
| Mn             | 3.0     |
| B              | 0.5     |
| H <sub>2</sub> | 0.001   |
| N <sub>2</sub> | 0.003   |

the balance iron with usual impurities. These wear plates gave more than a 300% increase in wear life as com-

pared with the previously used ferrous alloy having abrasion and wear resistant properties.

### EXAMPLE II

Plow scraper castings having a section size of  $1\frac{1}{2}$ " and weighing approximately 60 pounds each were cast from an alloy of the composition:

|                | Percent |
|----------------|---------|
| C              | 3.45    |
| Si             | 2.60    |
| Mn             | 3.2     |
| B              | 0.5     |
| H <sub>2</sub> | 0.001   |
| N <sub>2</sub> | 0.004   |

the balance iron with usual impurities. These plow scraper castings were used to divide hard abrasive materials from the inside perimeter of the rotary pan to a position under the mullers. The resulting life was from 300% to 500% greater than the ferrous alloy castings previously used for this purpose which were a carbide acicular ferrous matrix interspersed with flake or graphite carbide.

The cast alloy of this invention may have the following broad range of composition.

|                | Percent   |
|----------------|-----------|
| C              | 2.50-3.60 |
| Si             | 1.50-2.60 |
| Mn             | 0.30-4.5  |
| B              | 0.1-1.0   |
| H <sub>2</sub> | .001-.002 |
| N <sub>2</sub> | .001-.008 |

Chromium, molybdenum, nickel and copper may be present alone or together in small amounts with iron making up the balance of the composition.

A preferred somewhat narrower range of composition is:

|    | Percent   |
|----|-----------|
| C  | 3.30-3.60 |
| Si | 2.20-2.60 |
| Mn | 0.75-4.5  |
| B  | 0.1-1.0   |

with the remaining materials as mentioned herein above.

### EXAMPLE III

Screen plates with discharge apertures varying from  $\frac{3}{4}$ " to  $\frac{1}{16}$ " and section sizes from  $\frac{1}{2}$ " to 1" and averaging 150 pounds in weight were cast from the alloy of Example I. Abrasive materials were discharged through these

plates from a rotary muller. The resulting screen life was in excess of 300% greater than that of the previously used plates.

In the foregoing specification I have set out certain preferred embodiments of this invention, however, it will be understood that it may be otherwise embodied within the scope of the following claims.

I claim:

1. A manganese containing cast iron composition having unusual abrasive resistance and an oriented lamellar matrix consisting of at least one member from the group consisting of pearlite and bainite alternating with a complex carbide structure consisting of complex boron nitrides, boron carbides and other boron compounds consisting essentially of carbon about 2.50% to 3.60%, silicon about 1.50% to 2.60%, manganese 0.3% to 4.5%, boron 0.1% to 1.0% and the balance iron with usual impurities in ordinary amounts.

2. A cast iron composition as claimed in claim 1 wherein the alloy includes small amounts of nickel, chromium, copper and molybdenum.

3. A cast iron composition as claimed in claim 1 wherein the carbon is about 3.30% to 3.60% and the silicon is about 2.20% to 2.60%.

4. A manganese containing cast iron composition as claimed in claim 1 wherein the carbon content is 3.4%, the silicon content is 2.4%, the manganese content is 3% and the boron content is 0.5%.

5. A manganese containing cast iron composition as claimed in claim 1 wherein the carbon content is 3.45%; the silicon content is 2.6%, the manganese content is 3.2% and the boron content is 0.5%.

### References Cited

#### UNITED STATES PATENTS

|           |         |           |       |           |
|-----------|---------|-----------|-------|-----------|
| 2,046,912 | 7/1936  | Kormann   | ----- | 75-123 CB |
| 2,943,932 | 7/1960  | White     | ----- | 75-123 CB |
| 3,299,482 | 1/1967  | Tache     | ----- | 75-123 CB |
| 2,224,448 | 12/1940 | Schlumpt  | ----- | 75-123 B  |
| 2,630,382 | 3/1953  | Wasserman | ----- | 75-123 CB |
| 3,193,383 | 7/1965  | Butler    | ----- | 75-123    |
| 3,253,907 | 5/1966  | Schwindt  | ----- | 75-130    |

45 HYLAND BIZOT, Primary Examiner

U.S. Cl. X.R.

148-35